

Feb. 11, 1958

H. C. HAMPE

2,822,591

HOT TOP CASING

Filed Aug. 2, 1954

FIG.1.



FIG.3.



FIG.4.



FIG.5.



FIG.6.



FIG.7. FIG.8.



INVENTOR:

HARRY C. HAMPE

By *Drawings and Satherland*  
ATTORNEYS.

1

2,822,591

## HOT TOP CASING

Harry C. Hampe, University City, Mo., assignor to  
Oswald Refractories Company, Brentwood, Mo., a corporation of Missouri

Application August 2, 1954, Serial No. 447,331

2 Claims. (Cl. 22—147)

This invention relates to hot top casings.

It is customary to provide at the top of a vertical ingot mold a so-called hot top casing. The function of such a casing is to retard the cooling of molten metal at the upper end of the mold, so as to provide a reservoir of molten metal, feeding by gravity into the interstices of the cooling metal, in order to produce a sound and solid ingot. The preservation of a molten pool at the top also permits dross to rise to the top. Traditionally, such hot top casings rest on top of the mold and are destroyed when the ingot is removed from the mold.

It has been proposed heretofore to construct an ingot mold with an enlarged cavity or recess at its upper end, the base of the recess being defined by an annular shoulder, and to line the enlarged cavity with refractory blocks supported by the shoulder. However, these prior art insert-type refractory hot top casings have also had a very limited life, having to be replaced after one to four pourings, because they have broken under the strains exerted upon them, and molten metal has made its way into joints between the various blocks.

One of the objects of this invention is to provide a refractory hot top casing which is capable of repeated use without replacement, and which can be tightly fitted into a roughly finished mold cavity enlargement.

Other objects will become apparent to those skilled in the art in the light of the following description and accompanying drawing.

In accordance with this invention, generally stated, a refractory hot top casing is provided for use in an ingot mold having an enlarged top cavity or recess the base of which is defined by an annular shoulder. The refractory hot top is made sectionally, with wedge-shaped corner blocks by which the casing may be tightened so as to present an unbroken surface to the metal in the mold and to accommodate any irregularities in the walls of the recessed portion of the mold.

In the drawing,

Figure 1 is a top plan view of an ingot mold in which a refractory hot top casing, constructed in accordance with one embodiment of this invention, is installed;

Figure 2 is a sectional view taken along the line 2—2 of Figure 1;

Figure 3 is a top plan view of a wall block of the hot top casing shown in Figures 1 and 2;

Figure 4 is a view in end elevation of the wall block shown in Figure 3;

Figure 5 is a view in front elevation of the wall block shown in Figure 3;

Figure 6 is a plan view of a corner wedge block of the hot top casing shown in Figures 1 and 2;

Figure 7 is a view in front elevation of the wedge block shown in Figure 6; and

Figure 8 is a view in side elevation of the wedge block shown in Figure 6.

Referring now to the drawing for an illustrative embodiment of this invention, reference numeral 1 indicates an ingot mold having a mold cavity 2. The mold cavity

2

2 consists of an upper cavity 3 and a lower cavity 4. The upper cavity 3 is larger laterally than the upper end of the lower cavity 4, so that an annular shoulder 6 is provided at the juncture of the lower cavity 4 and the upper cavity 3. The upper cavity 3 is approximately square in cross-section, being defined by plane walls 7, substantially perpendicular to one another, and by rounded corners 5 connecting contiguous walls.

Resting on the shoulder 6, and extending through the height of the upper cavity 3 is a hot top casing 10 of this invention. The hot top casing 10, in the embodiment shown, is made in twelve parts. Along each of the four flat sides 7 of the upper cavity are a left-hand wall block 12, shown in detail in Figures 3 through 5, and a right-hand wall block 14 which is a mirror image of the left-hand wall block 12.

Each of the left-hand wall blocks 12 has a substantially vertical plane back 16, a flat end 17, a front face 18 which inclines toward the back 16 downwardly, a chamfered section 20 between the flat end 17 and front face 18 and a square end 15.

Similarly, the right-hand block 14 has a vertical back 26, a flat end 27, a front face 28 which inclines toward the back 26 downwardly, a chamfered section 30 between the flat end 27 and front face 28 and a square end 25. The square ends 15 and 25 abut one another tightly.

The chamfered sections 20 and 30 are wide at their tops and taper along the front faces 18 and 28. Thus the front faces 18 and 28 are wider at their bottom than at their top, as shown in Figures 4 and 5.

In each corner between the wall blocks 12 and 14 of contiguous sides is a corner wedge block 40. Each of the wedge blocks 40 has a flat vertical back 41, a front face 42 which inclines toward the back 41 downwardly, and sides 43 and 44, extending convergently from the back 41 to the front face 42. Thus the corner blocks 40 are wedge-shaped both in plan view and in side elevation. The corner wedge blocks may be made in different widths, so that if an upper mold cavity is oversize or undersize, or is slightly out of square, one or more wide or narrow corner wedge blocks may be used to give a tight fit.

The wall blocks 12 and 14 and the wedge blocks 40 are of the same height, and are flat on the top and bottom. The arris between the back of each of the blocks and its bottom is preferably chamfered as shown at 46 in Figures 4 and 8.

The downward convergence of the front faces of the wall and wedge blocks is preferably substantially the same as the downward outward flair of the lower cavity 4, and the width of the blocks at their lower ends is the same as the width of the shoulder 6, so that the front faces of the blocks form substantially uninterrupted continuations of the walls of the lower cavity 4, as indicated in Figure 2.

In preparing an ingot mold for use, the wall blocks 12 and 14 are placed in position as shown in Figure 1, with their square ends 15 and 25 abutting. The corner wedge blocks 40 are then inserted with their backs 41 as close to the corners of the upper cavity 3 as possible, so as to give the greatest possible amount of clearance between them and the wall blocks. The wedge blocks 40 are then pushed inwardly toward the center of the mold cavity as far as they will go. As the wedge blocks 40 are moved inwardly, the flaring sides 43 and 44 engage the chamfered sections 20 and 30 of wall blocks 12 and 14 and force the wall blocks 12 and 14 into tight abutment. Any spaces between the wedge blocks 40 and the wall blocks 12 and 14, and between the walls 7 of the upper cavity 3 and any of the blocks, are grouted.

It can be seen that other arrangements of wall blocks

and wedge blocks may be used. The preferred embodiment described is convenient to make and to install and produces excellent results. It is more flexible than other arrangements, and is less liable to breakage both in installation and in use. However, the wall blocks 12 and 14 may be made in one piece. This increases the danger of cracking and also increases the weight of the block to the point where it is somewhat difficult to handle. It is also possible to make the hot top casing in four pieces with two L-shaped blocks, and wedge blocks in two diagonally-opposite corners. However, this latter embodiment is, for most purposes, impractical in that the L-shaped blocks are difficult to manufacture, inordinately heavy, and liable to break from the strains set up in use.

The wall blocks and wedge blocks of the hot top casing of this invention are preferably made of refractory clays having low density, slag resistant and thermal shock resistant characteristics. First quality or better fire clay may be used. However, those skilled in the refractories art will understand that proper blends of first quality, super-duty or special super-duty refractory clays can be made up to have the particular characteristics desired. In actual practice, dry press, super-duty grade fire clay blocks used in casings of this invention have consistently been used for sixteen to twenty pours. High burned super-duty fire clay blocks, fired at approximately 2750° F., will also give excellent results.

While the particular dimensions form no part of this invention, the following detailed description will serve to illustrate a practical device.

In an ingot mold 75 inches high, 32 inches square at the bottom and 30 inches square at the top, with a mold cavity tapering from 20 $\frac{1}{4}$  inches square at the bottom to 19 $\frac{1}{2}$  inches square at the shoulder, and with a recess 15 inches high and 23 $\frac{3}{4}$  inches square, leaving a shoulder approximately 2 $\frac{1}{2}$  inches wide, the following dimensions have been found to be satisfactory for the blocks of the hot top casing:

| Wall blocks:                                             | Inches          |
|----------------------------------------------------------|-----------------|
| Height of blocks                                         | 15              |
| Thickness of blocks at base (without the bottom chamfer) | 2 $\frac{5}{8}$ |
| Thickness at top                                         | 3 $\frac{3}{4}$ |
| Thickness of flat end                                    | 1 $\frac{1}{4}$ |
| Width of bottom chamfer                                  | 1 $\frac{1}{2}$ |
| Width of chamfer section between front and flat end:     |                 |
| At top                                                   | 3               |
| At bottom                                                | 1 $\frac{3}{4}$ |
| Width of front face between square end and chamfer:      |                 |
| At top                                                   | 6 $\frac{1}{2}$ |
| At bottom                                                | 7 $\frac{1}{8}$ |
| Width of back                                            | 8 $\frac{3}{8}$ |
| Wedge blocks:                                            | Inches          |
| Height                                                   | 15              |
| Thickness at base                                        | 3               |
| Thickness at top                                         | 4 $\frac{1}{4}$ |
| Width of back                                            | 2 $\frac{3}{4}$ |
| Width of front face:                                     |                 |
| At top                                                   | 1 $\frac{3}{4}$ |
| At bottom                                                | 2               |
| Width of sides:                                          |                 |
| At top                                                   | 4 $\frac{1}{4}$ |
| At bottom                                                | 3               |

Numerous variations in the construction of the hot top

casing of this invention within the scope of the appended claims will be apparent to those skilled in the art, in the light of the foregoing disclosure. While in the illustrative embodiment shown, the ingot mold is substantially 5 square in cross-section, the hot top casing of this invention may be used in ingot molds of other shapes. For example, rectangular ingot molds having two long sides and two short sides, as compared with the square mold, are presently being used. In order to adapt the hot top 10 casing of this invention to such a mold, it is only necessary to increase the width of the wall blocks positioned along the long sides and to decrease the width of the wall blocks along the short sides. The use of a plurality of wall blocks along each side makes the hot top casing of this invention readily adaptable to various shapes, since individual wall blocks may be made of various different widths and configurations, so long as they are provided with camming end surfaces. So also, the configuration of the wedge blocks may be changed, so long as they are 15 so constructed as to perform their wedging function.

Having thus described the invention, what is claimed and desired to be secured by Letters Patent is:

1. In an ingot mold having an enlarged upper mold cavity, defined by generally flat walls and an internal 20 annular shoulder, a refractory hot top casing comprising: wall blocks resting on said shoulder and extending along the walls defining the sides of the enlarged mold cavity but terminating short of the meeting corners thereof; said 25 wall blocks having a plane substantially rectangular vertical back, a front face extending convergently downwardly toward said back, and a chamfered section of uniform angularity from top to bottom with respect to the said back, said chamfered section extending along the inner edge of the wall block adjacent the corner of the 30 enlarged mold cavity; and corner wedge blocks, in corners of said enlarged cavity between the chamfered sections of adjacent wall blocks; said corner wedge blocks having a substantially rectangular flat back, a front face which extends convergently downwardly toward the flat back and 35 sides which diverge in a direction away from the interior of the enlarged mold cavity, said sides being of uniform angularity with respect to the back of the corner wedge blocks, there being sufficient clearance between the back of the corner wedge blocks and the wall of the enlarged 40 mold cavity to permit the insertion of the wedge blocks after the wall blocks are in place, the divergence of the sides of the wedge blocks permitting them to bear against the chamfered sections of the wall blocks when the corner wedge blocks are moved inwardly, so that the wall blocks 45 and wedge blocks constituting the hot top casing are 50 forced tightly together.

2. A refractory hot top casing of the character described in claim 1 wherein the wall blocks along each wall are made up of a left-hand block and a right-hand block, 55 said left- and right-hand blocks being mirror images of one another, with abutting square ends opposite the flat ends adjacent the corners of the enlarged upper mold cavity.

60 References Cited in the file of this patent

UNITED STATES PATENTS

|           |         |               |
|-----------|---------|---------------|
| 1,804,205 | Charman | May 5, 1931   |
| 2,046,043 | Urmetz  | June 30, 1936 |
| 2,433,175 | Urmetz  | Dec. 23, 1947 |

65 FOREIGN PATENTS

|         |               |               |
|---------|---------------|---------------|
| 689,465 | Great Britain | Mar. 25, 1953 |
|---------|---------------|---------------|